

Sept. 18, 1956

J. ROCKOFF

2,763,033

TEXTILE COT

Filed Dec. 13, 1952



Fig. 1



Fig. 2

INVENTOR.  
JOSEPH ROCKOFF

BY  
*Joseph Rockoff*  
ATT'Y.

2,763,033

## TEXTILE COT

Joseph Rockoff, Dayton, Ohio, assignor to The Dayton Rubber Company, a corporation of Ohio

Application December 13, 1952, Serial No. 325,796

6 Claims. (Cl. 19—143)

This invention relates to textile machine units, and more particularly to cots or roll covers for spinning rolls. 15

A textile roller as used in present day drawing, roving and spinning machines, comprises a metal arbor having a sleeve-like roll cover known as a cot, surrounding the arbor. This cover is made of leather, cork composition, or certain types of rubber compounds.

In the past, most textile cots were made of leather. These cots proved to be not too satisfactory for use on modern machines which work at relatively high speeds, due to poor resistance to "lapping-up" and "eyebrowning" and due to their relatively short life. More recently, cots have been made of synthetic materials which show considerably longer life than leather, and also possess better resistance to "lapping-up" and "eyebrowning."

Despite the improved characteristics which have been imparted to textile cots by the use of some of the new types of synthetic rubber, these cots still do not function perfectly under all conditions and for all types of fibers. Some of the newer types of cots, although considerably improved over leather, still exhibit a tendency toward eyebrowning. This condition results from the failure of the cot to carry short fibers or "clearer waste" to the top clearer in order to gather properly. Instead, these short fibers collect at the outside edge of the top clearer and hang down over the roll. This condition is called "eyebrowning" and the mass of fibers which hangs down is called an "eyebrow." As the size of the "eyebrow" increases it will touch the yarn and bunches of short fibers will be pulled into the yarn, thus impairing its quality.

In applicant's prior application Serial No. 270,805, filed February 9, 1952, he has described a novel textile cot having incorporated therein polyvinyl alcohol to effect modification of the drafting properties thereof.

In applicant's co-pending application Serial No. 299,841, filed July 19, 1952, he has disclosed and described another type of improved textile drafting cot composition having incorporated therewith granulated shells of nut-like materials, such as peanut shells or almond shells. Cots made of the compositions referred to in the foregoing co-pending applications have been found to perform extremely well in service and to be highly resistant to eyebrowning and lapping-up. It has been applicant's experience, however, that even improved compositions of the foregoing type will eventually begin to lose their non-eyebrowning characteristics with the result that they will either have to be reground or the covers thereof replaced. Applicant has carried out extensive experiments to improve the surface life of textile cots and prolong the period of use before lapping-up or eyebrowning begins to occur in such cot.

In accordance with the present invention, applicant has discovered that highly improved characteristics with respect to durability and performance and particularly with respect to resistance to eyebrowning and lapping-up are obtained by incorporating in the cot compound both the polyvinyl alcohol and the ground up nut shells. The resulting product has been found to perform considerably

better than the cots made in accordance with the prior inventions having either polyvinyl alcohol or ground up nut shells alone as the modifying constituent. The present invention, therefore, is a continuation-in-part of my 5 prior application Serial No. 270,805, filed February 9, 1952, and of my prior application Serial No. 299,841, filed July 19, 1952.

As set forth above, it is therefore an object of the present invention to provide an improved textile roll cover or cot which will substantially eliminate objectionable eyebrowning and will at the same time provide excellent wear and resistance to lapping up of fibers.

Other features and advantages will become more readily apparent in the following description:

As described in the co-pending applications referred to above, applicant has discovered that by the incorporation of either polyvinyl alcohol or ground up shells in a cot composition the basis of which is an oil-resistant synthetic rubber-like material, eyebrowning is substantially eliminated during the useful life of the cot and the cot possesses excellent performance characteristics with respect to endurance and resistance to lapping up. Furthermore, these cots tend to work clearer waste back into the goods so that it is worked into the yarn thus eliminating a waste which would otherwise occur. Polyvinyl alcohol is normally obtained as a solid material and is incorporated in the cot compound as a granular material or powder by milling or otherwise, together with the ground shell and other compounding ingredients as normally utilized. The resulting compounded mixture is then extruded in tubular form, placed on a core, rag wrapped, and vulcanized. After vulcanization the rag wrap is removed and the resulting product ground to the desired size. The tube is then cut to the desired length to form cots or roll covers and these are then mounted on the arbor. A finish grind may be used before the cot is placed in operation. A preferred type of synthetic rubber in which this material is incorporated is an oil-resistant copolymer of the butadiene-acrylic nitrile type also known as Buna-N, Perbunan, GR-A, or by other well-known terms used in the trade. Although the butadiene-acrylic nitrile copolymers are preferred, other oil-resistant types of synthetic rubber, such as the polyhaloprenes (polychloroprene), and the like may be used. As is well known to the art, polyvinyl alcohol which is referred to herein, is a product obtained by the hydrolysis of polyvinyl acetate. The resulting compound is in the form of a solid gel which will vary in physical properties depending on the degree of hydrolysis to which the acetate has been subjected. The various conventional types of polyvinyl alcohol ranging from partially hydrolyzed to substantially completely hydrolyzed types have been found to function satisfactorily in applicant's composition. The nut shells used must be of a soft, porous and fibrous structure, 35 the most common examples of which are the shells of peanuts and almonds. The proportions of the respective materials which may be used has been found to be quite variable and in fact improved results are obtained even by the use of small amounts of both of the materials referred to. Therefore, the lower limit is that proportion at which a noticeable improvement will result which may be as low as one per cent of each. The upper limit of proportions is also not critical, although as a practical matter it is undesirable to utilize a combined proportion of these 50 materials which would be greater than double the weight of rubber in the compound. A preferred range of proportions is from 10 to 100 parts of the polyvinyl alcohol by weight for each 100 parts of the synthetic rubber and from 10 to 100 parts by weight of the ground shell material per 100 parts of synthetic rubber.

In the case of the polyvinyl alcohol the particle size is not critical but large size particles should be avoided

in order to insure uniform mixing, preferably a particle size is chosen which will pass through a 60 mesh sieve. In the case of ground nut shell material, the particle size is generally preferred to be in the range of about 20 to 60 mesh, but here too the limiting factor as to size is that which will insure uniform mixing on the mill.

The appended drawing illustrates a typical cot construction of the present invention.

In the drawing:

Figure 1 shows a view in elevation partly in cross section of a conventional type of double cot mounted on an arbor.

Figure 2 illustrates in cross section an enlarged view of a portion of a cross section of the cover shown in Figure 1.

In Figure 1 the double arbor is represented by 10, each side of the arbor having roll covers 11 and 11a mounted thereon. The particles 13 of ground shell material and 14 of polyvinyl alcohol which are embedded in the composition, are exposed at the surface of the roll as shown more clearly in Figure 2.

The following example will illustrate a typical cot compound of the type described above:

|                                                                | Parts by weight |
|----------------------------------------------------------------|-----------------|
| Perbunan (74% butadiene 26% acrylonitrile emulsion copolymer)  | 100             |
| Plasticizer and tackifier, phenolformaldehyde resin (Bakelite) | 10-20           |
| Sulfur                                                         | 5               |
| Accelerator (mercaptobenzothiazole or the like)                | 1-2             |
| Zinc oxide                                                     | 8-12            |
| Clay filler                                                    | 15-35           |
| Diphenylguanidine                                              | 0.25            |
| Ground peanut shells particle size 40 mesh                     | 50              |
| Polyvinyl alcohol (98.5-100% hydrolyzed) (Elvanol)             | 20              |

The ingredients corresponding to the foregoing recipe were mixed, extruded, vulcanized, and made into cots in the manner described above. The resulting cots were then placed on spinning frames drafting cotton and rayon fibers in comparison with other cots of similar Perbunan compounds, but without both the polyvinyl alcohol and the peanut shell. Cot A was made as above, but eliminated the polyvinyl alcohol and contained 50 parts of ground peanut shell per 100 parts by weight of the rubber. Cot B eliminated the peanut shell, but contained 40 parts of polyvinyl alcohol per 100 parts by weight of the rubber. Cot C was made according to the above compound and contained 50 parts of peanut shell and 20 parts of polyvinyl alcohol per 100 parts by weight of the rubber. These cots were placed on spinning and drawing frames in a mill and were operated spinning and drawing both cotton and rayon fibers.

Cot A, after 24 weeks of operation in spinning, continued to perform satisfactorily. In drawing, the cots began eyebrowing after 156 hours.

Cot B, after 24 weeks of operation in spinning, continued to operate satisfactorily with cotton, but began to eyebrow with rayon. In drawing, the cots began to eyebrow after 29 hours.

Cot C, after 24 weeks of operation in spinning, con-

tinued to operate satisfactorily on both cotton and rayon. In drawing, after 286 hours of continuous operation, no signs of eyebrowing were observed.

The superior performance of cot C was clearly demonstrated.

In a further comparison, cots similar to cot C were run on a high speed experimental drawing frame run at speeds double those used in the mills, and tested for eyebrowing in drawing cotton and rayon fibers. Plain Perbunan cots without the ground shell and polyvinyl alcohol were also run, along with Perbunan cots containing 50 parts by weight of ground cork per 100 parts of rubber. The plain Perbunan cot began to eyebrow after 15 minutes of operation, the cork-containing cots

began to eyebrow after 70 hours, while the ground shell-polyvinyl alcohol cots were continuing to run without eyebrowing after 120 hours.

I claim:

1. A textile fiber drafting cot having a working surface composed of a vulcanized oil-resistant synthetic rubber-like material having intimately incorporated therewith discrete particles of polyvinyl alcohol and particles of the soft, porous and fibrous shells of a nut-like material, to effect modification of the drafting properties thereof.

2. A cot according to claim 1 wherein the shell particles are ground up peanut shells.

3. A cot according to claim 2 wherein the synthetic rubber-like material is a butadiene-acrylonitrile copolymer.

4. A textile fiber drafting cot according to claim 3 wherein the synthetic rubber-like material is a poly-chloroprene.

5. A textile fiber drafting cot having a working surface composed of a vulcanized oil-resistant synthetic rubber-like material having intimately incorporated therewith from about 10 to about 100 parts by weight of discrete particles of polyvinyl alcohol per 100 parts of a synthetic rubber-like material and from about 10 to about 100 parts by weight of particles of the soft, porous and fibrous shells of a nut-like material per 100 parts of the synthetic rubber-like material by weight.

6. A textile cot according to claim 5 wherein the synthetic rubber-like material is a butadiene-acrylonitrile copolymer.

#### References Cited in the file of this patent

#### UNITED STATES PATENTS

|           |             |                |
|-----------|-------------|----------------|
| 2,304,656 | Rockoff     | Dec. 8, 1942   |
| 2,373,698 | McGeary     | Apr. 17, 1945  |
| 2,414,803 | D'Alelio    | Jan. 28, 1947  |
| 2,450,410 | Baymiller   | Oct. 5, 1948   |
| 2,482,237 | Berglund    | Sept. 20, 1949 |
| 2,570,935 | Freedlander | Oct. 9, 1951   |
| 2,645,587 | Williamson  | July 14, 1953  |

#### FOREIGN PATENTS

|           |               |                |
|-----------|---------------|----------------|
| 15,988    | Great Britain | of 1915        |
| 511,489   | Great Britain | Aug. 18, 1939  |
| 579,083   | Great Britain | July 23, 1946  |
| 643,764   | Great Britain | Sept. 27, 1950 |
| 1,000,963 | France        | Oct. 17, 1951  |